

## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## PROCESS OF PULPING RAW CELLULOSIC MATERIAL

No Drawing.

Application filed June 1, 1928. Serial No. 282,276.

In the pulpmaking industry, the chemical digesters and the hazard incident to their pulping of raw cellulosic materials such as wood has heretofore been carried on by batch operation. For instance, it is the usual practice to charge a digester with chipped wood and cooking liquor, and then to close the digester and to cook the charge at elevated temperature and under pressure until fiber liberation has been effected. The reason for this practice is apparently due to the fact that the encrusting or cementitious content of the wood can be dissolved by the cooking liquor only at temperatures materially above 212° F., and in order to attain such temperatures it is necessary to maintain the liquor under sufficient pressure to raise its boiling point to or above such temperatures. Apparently, the pressure maintained during cooking has no function other than permitting the attainment of fiber-liberating temperatures, for if chipped wood be digested at 212° F., for instance in a cooking liquor such as ordinarily employed in kraft digestion, fiber liberation will not be effected, even if a pressure in the order of magnitude of 100 pounds be maintained during digestion.

I have discovered that raw cellulosic material such as wood may be pulped under atmospheric pressure if a cooking liquor of a composition permitting the attainment of fiber-liberating temperatures be employed. In producing a cooking liquor of this character, I dissolve in the liquor a water-soluble or water-miscible body in amount to raise its boiling point sufficiently to permit reaching fiber-liberating temperatures. The bodies which I employ do not undergo decomposition at such temperatures, nor do they injure the resulting pulp. Various bodies are available for this purpose,—ethylene glycol, and/or glycerol, or other polyhydric alcohols, for instance, being especially suitable, as they may be readily recovered from the spent cooking liquor, as by steam distillation. One of the major advantages of a process such as described is that the pulping of raw cellulosic materials such as wood may be carried out continuously in open tanks, thereby eliminating the necessity of expensive high pressure

While the process of the present invention may be applied when using liquors of acid, neutral, and alkaline character, it is especially applicable to quick-cooking processes where batch operation involves a greater loss of time than in slow-cooking processes. For instance, the process of the present invention may be applied advantageously when wood is being pulped by an alkaline process of digestion such as the soda process, or the kraft process, so-called.

In preparing cooking liquors such as I employ according to the process of the present invention, the fiber-liberating chemical may be used in substantially the same amount as in ordinary cooking liquors, but a portion of the water usually employed is replaced by an amount of water-soluble or water-miscible body sufficient to permit the attainment of fiber-liberating temperatures under atmospheric pressure. The temperature range for fiber liberation without injuring the pulp is from about 250° to about 350° F., so that if glycerol is used for raising the boiling point of the liquor, it should be added in amount varying from about 80% to about 96% of the weight of the water employed. One of the advantages of using glycerol, is that it does not react with the fiber-liberating chemical or undergo decomposition, even when raised to its boiling point, and in no way injures the raw cellulosic material or the resulting pulp. Furthermore, a substantial proportion of the spent liquor resulting from digestion may be reused, while glycerol present in the rest of the spent liquor may be readily recovered as by steam distillation. After distillation, the residual liquor is highly concentrated in spent chemical, so that recovery of the chemical therefrom may be effected without concentrating such liquor. In other words, after glycerol has been steam-distilled from the spent liquor, the residual liquor containing the spent chemical may be introduced directly into a furnace wherein its organic content is burned and its inorganic content converted into smelted compounds which may

be dissolved in water and used for the preparation of fresh cooking liquor.

One procedure which gave satisfactory results in actual practice was carried out substantially as follows. White birch in the form of  $\frac{1}{4}$ " chips and a liquor consisting of a mixture of 10% water and 90% glycerol and containing 3.0 pounds of alkali per cubic foot of liquor, figured on the basis of Na<sub>2</sub>O equivalent, were charged into open tanks. The liquor was of 35% sulphidity and so was substantially similar in its content of fiber-liberating chemical to the usual kraft liquors. The charge was gradually heated to fiber-liberating temperatures, digestion being continued over a period of about six hours between about 238° to 300° F. At the end of this time, a good yield of pulp having about the same color, strength, and tear resistance as the usual kraft pulp was obtained.

Various liquors other than that given in the foregoing example, of greater or less alkalinity and/or sulphidity, may be employed according to the present invention, to produce pulps of various physical and chemical characteristics. So, too, other kinds of wood, such as spruce and poplar, may be employed as the raw material, and fiber liberation effected under somewhat different time and temperature conditions.

The pulp may be separated or washed free from the spent liquor of digestion. A portion of the spent liquor, say about 50%, may be reused together with fresh cooking liquor, and the remaining liquor subjected to steam distillation for the recovery of glycerol for reuse in the preparation of fresh cooking liquor. The spent chemical remains dissolved in the aqueous residue left in the still. This residue, being highly concentrated in chemical, may be delivered directly into a recovery furnace wherein its combustible content is burned and its inorganic content smelted to produce a smelt of the desired composition. The smelt may be dissolved in water and used in the preparation of fresh cooking liquors.

Having thus described certain embodiments of this invention, it is evident to those skilled in the art that various changes and modifications might be made therein without departing from the spirit or scope of invention as defined in the appended claims.

What I claim is:

- 55 1. A process of pulping raw cellulosic material, which comprises digesting such material under atmospheric pressure and at temperatures materially above 212° F. in an aqueous cooking liquor comprising fiber-liberating chemical and a water-miscible body permitting the attainment of such temperatures at such pressure.
- 60 2. A process of pulping raw cellulosic material, which comprises digesting such material under atmospheric pressure at tem-

peratures of about 250° F. to 350° F. in an aqueous cooking liquor comprising a fiber-liberating chemical and a water-miscible body permitting the attainment of such temperatures at such pressure.

70 3. A process of pulping raw cellulosic material which comprises digesting such material under atmospheric pressure and at fiber-liberating temperatures in an aqueous cooking liquor comprising fiber-liberating 75 chemical and glycerol in amount sufficient to permit the attainment of such temperatures at such pressure.

80 4. A process of pulping raw cellulosic material, which comprises digesting such material under atmospheric pressure and at fiber-liberating temperatures in a cooking liquor comprising a mixture of water and glycerol containing fiber-liberating chemical, separating the resulting pulp from the spent liquor, and recovering glycerol from such spent liquor for the preparation of fresh cooking liquor.

85 5. A process of pulping raw cellulosic material, which comprises digesting such material under atmospheric pressure and at fiber-liberating temperatures in a cooking liquor comprising a mixture of water and glycerol containing inorganic fiber-liberating chemical, separating the resulting pulp from the spent liquor, and steam-distilling glycerol from such spent liquor and recovering the valuable inorganic content from the remaining aqueous liquor for the preparation 90 of fresh cooking liquor.

95 6. A process of pulping raw cellulosic material, which comprises digesting such material under atmospheric pressure and at fiber-liberating temperatures in an alkaline cooking liquor comprising a mixture of water and glycerol having a fiber-liberating chemical content substantially similar to that of a kraft cooking liquor, separating the resulting pulp from the spent liquor, and steam-distilling glycerol from such spent liquor and smelting the valuable inorganic content of the remaining aqueous liquor for the preparation 100 of fresh cooking liquor.

105 In testimony whereof I have affixed my signature.

110 GEORGE A. RICHTER.

115

120

123

130